# EUROPEAN PATENT SPECIFICATION

(11) **EP 0 030 249 B1**
(45) Date of publication and mention of the grant of the patent: **20.07.1983**
(21) Application number: 79302746.7
(22) Date of filing: 30.11.1979
(51) Int. Cl.: C10G 29/20, H01B 3/22

(54) **Insulating oil compositions**
Isolierölzusammensetzungen
Compositions d'huile isolante

(43) Date of publication of application: 17.06.1981
(73) Proprietor: GULF RESEARCH & DEVELOPMENT COMPANY, Pittsburgh Pennsylvania 15230 (US)
(72) Inventor: Schulz, Johann G. D., Pittsburgh, Pennsylvania 15208 (US); Onopchenko, Anatoli, Monroeville, Pennsylvania 15146 (US); Kofke, William A., Irwin, Pennsylvania 15642 (US)
(74) Representative: Huskisson, Frank Mackie

## Description

### Insulating oil compositions

### Background of the invention

### 1. Field of the invention

This invention relates to novel insulating oil compositions comprising a major amount of an insulating oil and a minor amount of a product obtained as a result of a process which comprises reacting benzene with ethylene in the presence of an alkylation catalyst to obtain a reaction mixture containing largely unreacted benzene, ethylbenzene, polyethylbenzenes, 1,1-diphenylethane and heavier material, separating at least benzene, ethylbenzene and polyethylbenzenes from said reaction mixture and thereafter recovering from said heavier material a fraction whose boiling points fall within a temperature range of about 255° to about 420°C as said product.

### 2. Description of the prior art

Insulating oils, for example, transformer oils, are required to have low power factors and high dielectric strengths, and to be able to maintain thermal and oxidative stability toward degradation and oxidation and to possess minimum tendency toward the formation of gas while in use. See, for example, U.S. Patent No. 3,549,537 to Brewster et al. Insulating oils composed largely of naphthenes and/or highly-branched, non-cyclic, paraffins can be used satisfactorily as transformer oils, for example, but unfortunately, they possess the tendency to produce gas during service.

### Summary of the invention

We have found that the gassing characteristics of insulating oils composed largely of naphthenes and/or highly-branched, noncyclic paraffins can be greatly decreased by the addition thereto of a selected amount of a product obtained as a result of a process which comprises reacting benzene with ethylene in the presence of an alkylation catalyst to obtain a reaction mixture containing unreacted benzene, ethylbenzene, polyethylbenzenes, 1,1-diphenylethane and heavier material, separating at least benzene, ethylbenzene and polyethylbenzenes from said reaction mixture and thereafter recovering from said heavier material a fraction whose boiling points fall within a temperature range of 255° to 420°C as said product.

### Brief description of novel insulating oil compositions

The insulating oils used herein can be obtained from any naphthenic and/or paraffinic origin. By "naphthenic and/or paraffinic oils" we mean to include naturally-derived, or synthetic, stocks containing largely one-ring structures, such as cyclopentane and cyclohexane derivatives, two-ring structures, such as decalin and dicyclohexyl derivatives, three-, four-, and five-membered ring structures, which may be part of the same or different molecule and their mixtures, etc. The paraffinic oils are defined as being largely of highly-branched, non-cyclic, compounds. A more useful conventional definition is that developed by E. C. Lane and E. L Garton in the "Bureau of Mines Report of Investigations No. 3279", September, 1935, and reported in "Petroleum Refining Processes" by M. M. Stephens and 0. F. Spencer, 4th Edition, The Pennsylvania State University Press, University Park, Pa., 1958, page 38, in which classification is based on the gravity of the first two distillation cuts. Typical naphthenic crudes include those from Huntingdon Beach, San Joaquin, Coastal B-1, etc. Typical paraffinic crudes are the Poza Rica, Kuwait, Grand Bay/Quarantine Bay, Ordovician Crudes, etc. In addition these oils can be synthetic oils, such as those obtained as the result of the oligomerization of 1-olefins having from six to 14 carbon atoms, preferably from eight to 12 carbon atoms, such as 1- decene, mixtures of 1-decene and 1-octene, 1-dodecene, etc., as described, for example, in US-A-4,045,507 to Cupples et al. Mixtures of naphthenic and paraffinic oils, including mixtures of natural and synthetic oils, can also be used, for example, in weight ratios of about 99:1 to about 1:99, preferably about 90:10 to about 10:90. In general the insulating oil used herein can be defined in accordance with the parameters set forth in Table I.

The product that is added to the above insulating oils to reduce their gassing tendencies of such insulating oils are defined in EP-A-0000622 and 0000619 filed in the names of J. G. D. Schulz, C. M. Selwitz and A. Onopchenko. Briefly, the product is obtained by reacting benzene with ethylene to obtain a reaction mixture containing unreacted benzene, ethylbenzene, polyethylbenzenes, 1,1-diphenylethane and heavier material, separating at least benzene, ethylbenzene, and polyethylbenzenes from said reaction mixture and thereafter recovering from said heavier material the entire fraction, or any portion of said fraction, whose boiling points at atmospheric pressure (ambient pressure) fall within a temperature range of 255° to 420°C, preferably 260° to 400°C, most preferably 268° to 400°C. In case 1,1-diphenyl ethane is also removed from said heavier material the product that is added to the above insulating oils is the entire fraction, or any portion of said fraction, whose boiling points at atmospheric pressure fall within a temperature range of 275° to 420°C, preferably 280° to 400°C.

The amounts of said product added to the insulating oil to inhibit the gassing tendency thereof can be varied over a wide limit, but, in general, the amount present, based on the weight of the final insulating composition, will be in the range of five to 20 weight per cent, preferably five to 15 weight per cent. Since the insulating oil and said product are both hydrocarbons and therefore completely miscible one in the other, mixing of the two at ambient temperature and ambient pressure until a homogeneous solution is obtained will suffice.

### Description of preferred embodiments

The following Table 11 compares the properties of the naphthenic base oil employed herein with the ASTM D-3487 insulating oil specifications for Type I Oil. The naturally-derived base oil (naphthenic) was obtained from Interprovincial Pipeline No. 1 and was a mixture of low sulfur, low pour point crudes. After conventional distillation, the fraction consisting of a 50:50 mixture of light vacuum and heavy vacuum oils (Gravity °API 25) was subjected to hydrotreating following the conditions in US-A-3,764,518. The purpose of this treatment was to upgrade the product through hydrocracking, isomerization and saturation. After the first stage hydrotreatment, the product was then subjected to a second stage hydrotreatment following the conditions in CA-A-978,881, wherein the primary purpose of such treatment is to saturate aromatic structures with hydrogen. The product from the two stage hydrotreatment has the properties shown in Table II. The synthetic base oil was prepared in accordance with the procedure of Example 1 of US-A-4,045,507 of Cupples et al, employing 1- decene as feedstock. The product from this oligomerization, after stripping off unreacted 1-decene, indicated 53 per cent conversion, and was found to contain 24 weight per cent dimer, the remainder being the trimer, tetramer and pentamer of 1-decene. The total product was then passed over a commercial nickel catalyst (Ni0104T, 1/8-inch pellets having a surface area of 125 square meters per gram) at 165°C and 600 pounds per square inch gauge (41 kilograms per square centimeter) of hydrogen pressure at a rate sufficient to effect stabilization of the product through hydrogenation. Distillation under vacuum afforded the synthetic base oil used herein, a dimer fraction boiling in the temperature range of 160°-168°C at 666 Pa (five millimeters of mercury).

A product for adding to the naphthenic oil was prepared as follows: Benzene and ethylene in a molar ratio of 9:1 were contacted in the liquid phase, while stirring, in a reactor at a temperature of 130°C and a pressure of 70 pounds per square inch gauge (4.9 kilograms per square centimeter) in the presence of AICI₃ catalyst over a period of one hour, which was sufficient to convert all of the ethylene. The AICI₃ complex catalyst was prepared by dissolving AICI₃ in a polyethylbenzene cut from a previous run so that after the addition the composition of the catalyst complex was as follows: 31.5 weight per cent AICI₃, 7.0 weight per cent benzene, 19.3 weight per cent ethylbenzene, 29.8 weight per cent polyalkylated benzenes, 3.4 weight per cent 1,1 1-diphenylethane and 9.0 weight per cent higher-boiling components. The amount of AICI₃ present in the catalyst mixture amounted to 0.0034 parts by weight per one part by weight of ethylbenzene produced. Also present in the catalyst was ethyl chloride as promoter in an amount corresponding 0.0034 parts by weight per one part by weight of ethylbenzene produced to maintain a high catalyst efficiency. Analysis of the alkylation product showed the presence of 49.0 weight per cent benzene, 32.9 weight per cent ethylbenzene, 17.5 weight per cent of polyalkylated benzenes (6.0 weight per cent diethylbenzene, 2.7 weight per cent triethylbenzenes, 2.1 weight per cent tetraethylbenzenes and 6.7 weight per cent other alkylbenzenes), 0.1 weight percent 1, 1-diphenylethane and 0.4 weight percent residue. The alkylation product was subjected to distillation to recover unreacted benzene, ethylbenzene, polyalkylated benzenes and 1,1-diphenyiethane, and the benzene and polyalkylated benzenes were recycled to the reaction zone. The residue remaining was a dark, viscous, high-boiling material, and was produced in an amount corresponding to 0.012 parts for each part of ethylbenzene produced. The residue so obtained was subjected to distillation to obtain a cut having a boiling point at atmospheric pressure within the temperature range of 275° to 400°C. This cut was the product added to the naphthenic oil and to the paraffinic oil in a later example. The incorporation of the product in the naphthenic oil was easily effected by physical blending, since each is miscible in the other in all proportions. Two blends were prepared, one containing 12 weight percent of the product from the residue (Blend No. 1) and the other 15 weight per cent (Blend No. 2). The results obtained are tabulated below in Table III.

The data in the above table clearly show the advantages resulting from the claimed invention. The base oil alone had a tendency to give off much gas. The mere addition of a portion of the residue from the reaction of benzene with ethylene to the base oil in fact not only greatly reduced gassing tendency of the oil but resulted in a blend having gas absorption properties. Note, too, the particularly surprising fact that the addition of inherently unstable additive to a base oil did not adversely affect the sludge and acid number and that the number of minutes when such blends were subjected to the rotary bomb oxidation tests was actually extended from 125 to at least 190. This is most unusual in light of the data in Table IV, below, which shows that the portion of the residue alone gave poor results when subjected to the Oxidation Test ASTM D-2440 and Rotary Bomb Oxidation Test ASTM D-2112. Other data in Table III show that a combination of base oil and residue from the reaction of benzene with ethylene not only gives good oxidative stability and low gassing tendencies, but that components in the mixture are compatible with each other as physical properties show.

Additional tests were carried out wherein the residue added to the naphthenic oil was also added to the synthetic oil defined above. For this purpose a mixture containing 90 weight per cent paraffin base oil and 10 weight per cent of residue was used (Blend III). The results obtained are set forth in Table V below.

The data in Table V show that a blend of residue from the reaction of benzene with ethylene and a paraffinic base oil has excellent oxidative stability, very low gassing tendency, and that the two fluids in a mixture are compatible with each other as physical properties show.

Obviously, many modifications and variations of the invention, as hereinabove set forth, can be made without departing from the spirit and scope thereof, and therefore only such limitations should be Imposed as are indicated in the appended claims.

## Claims

1. A novel insulating oil composition comprising a major amount of an insulating oil and a minor amount of a product obtained as a result of a process which comprises reacting benzene with ethylene in the presence of an alkylation catalyst to obtain a reaction mixture containing unreacted benzene, ethylbenzene, polyethylbenzenes, 1,1-diphenylethane and heavier material, separating at least benzene, ethylbenzene and polyethylbenzenes from said reaction mixture and thereafter recovering from said heavier material a fraction whose boiling points fall within a temperature range of 255° to 420°C as said product.

2. The composition of Claim 1 wherein said insulating oil is a naphthenic oil.

3. The composition of Claim 1 wherein said insulating oil is a paraffinic oil.

4. The composition of Claim 1 wherein said insulating oil is a paraffinic oil obtained from the oligomerization of 1-olefins having from six to 14 carbon atoms.

5. The composition of Claim 1 wherein said insulating oil is a paraffinic oil obtained from the oligomerization of 1-olefins having from eight to 12 carbon atoms.

6. The composition of Claim 1 wherein said insulating oil is a paraffinic oil obtained from the oligomerization of 1-decene.

7. The composition of Claim 1 wherein the amount of said product in the insulating oil composition is in the range of five to 20 weight per cent.

8. The composition of Claim 1 wherein the amount of said product in the insulating oil composition is in the range of five to 15 weight per cent.

9. The composition of Claim 1 wherein the boiling points of said fraction fall within a temperature range of 260° to 400°C.

10. The composition of Claim 1 wherein the boiling points of said fraction fall within a temperature range of 267°C to 400°C.

11. The composition of Claim 1 wherein the boiling points of said fraction fall within a temperature range of 275° to 420°C.

12. The composition of Claim 1 wherein the boiling points of said fraction fall within a temperature range of 280° to 400°C.

## Patentansprüche

1. Neue Isolierölzusammensetzung enthaltend einen größeren Anteil an einem Isolieröl und einen geringeren Anteil an einem Produkt, das man mittels eines Verfahrens erhält, bei dem man Benzol mit Ethylen in Gegenwart eines Alkylierungskatalysators zu einem Reaktionsgemisch umsetzt, das nichtreagiertes Benzol, Ethylbenzol, Polyethylbenzole, 1,1-Diphenylethan und schwereres Material enthält, daraus zumindest Benzol, Ethylbenzol und die Polyethylbenzole abtrennt und dann aus dem schwereren Material das Produkt als eine Fraktion gewinnt, die zwischen 255°C und 420°C siedet.

_{Öl} ist. ^{2.} Zusammensetzung Anspruch 1, dadurch gekennzeichnet, daß das Isolieröl ein naphthenisches

3. Zusammensetzung nach Anspruch 1, dadurch gekennzeichnet, daß das Isolieröl ein paraffinisches 01 ist.

4. Zusammensetzung nach Anspruch 1, dadurch gekennzeichnet, daß das Isolieröl ein paraffinisches Öl ist, das man durch Oligomerisation von 1-Olefinen mit 6 bis 14 Kohlenstoffatomen erhalten hat.

5. Zusammensetzung nach Anspruch 1, dadurch gekennzeichnet, daß das Isolieröl ein paraffinisches Öl ist, das man durch Oligomerisation von d 1-Olefinen mit 8 bis 12 Kohlenstoffatomen erhalten hat.

6. Zusammensetzung nach Anspruch 1, dadurch gekennzeichnet, daß das Isolieröl ein paraffinisches Öl ist, das man durch Oligomerisation von 1-Decen erhalten hat.

7. Zusammensetzung nach Anspruch 1, dadurch gekennzeichnet, daß die Menge an dem Produkt in der Isolierölzusammensetzung zwischen 5 und 20 Gew.-% beträgt.

8. Zusammensetzung nach Anspruch 1, dadurch gekennzeichnet, daß die Menge an dem Produkt in der Isolierölzusammensetzung zwischen 5 und 15 Gew.-% beträgt.

9. Zusammensetzung nach Anspruch 1, dadurch gekennzeichnet, daß die Siedepunkte der Fraktion innerhalb des Temperaturbereichs von 260 bis 400°C liegen.

10. Zusammensetzung nach Anspruch 1, dadurch gekennzeichnet, daß die Siedepunkte der Fraktion innerhalb des Temperaturbereichs von 267 bis 400°C liegen.

11. Zusammensetzung nach Anspruch 1, dadurch gekennzeichnet, daß die Siedepunkte der Fraktion innerhalb des Temperaturbereichs von 275 bis 420°C liegen.

12. Zusammensetzung nach Anspruch 1, dadurch gekennzeichnet, daß die Siedepunkte der Fraktion innerhalb des Temperaturbereichs von 280 bis 400°C liegen.

## Revendications

1. Nouvelle composition d'huile isolante, comprenant une quantité majeure d'une huile isolante et une quantité mineure d'un produit obtenu comme résultat d'un procédé qui comprend la réaction du benzène avec l'éthylène, en présence d'un catalyseur d'alkylation, pour obtenir un mélange réactionnel contenant du benzène n'ayant pas réagi, de l'éthylbenzène, des polyéthylbenzènes, du 1,1-diphényl- éthane et de la matière plus lourde, la séparation d'au moins le benzène, l'éthylbenzène et les polyéthylbenzènes de ce mélange réactionnel puis la récupération, à partir de ladite matière plus lourde, d'une fraction dont les points d'ébullition se situent dans une gamme de températures de 255° à 420°C, à titre dudit produit.

2. Composition selon la revendication 1, dans laquelle l'huile isolante est une huile naphténique.

3. Composition selon la revendication 1, dans laquelle ladite huile isolante est une huile paraffinique.

4. Composition selon la revendication 1, dans laquelle ladite huile isolante est une huile paraffinique obtenue à partir de l'oligomérisation de 1 -oléfines ayant de 6 à 14 atomes de carbone.

5. Composition selon la revendication 1, dans laquelle ladite huile isolante est une huile paraffinique obtenue à partir de l'oligomérisation de 1 -oléfines ayant de 8 à 12 atomes de carbone.

6. Composition selon la revendication 1, dans laquelle ladite huile isolante est une huile paraffinique obtenue à partir de l'oligomérisation de 1 -décène.

7. Composition selon la revendication 1, dans laquelle la quantité dudit produit dans la composition d'huile isolante se situe entre 5 et 20% en poids.

8. Composition selon la revendication 1, dans laquelle la quantité dudit produit dans la composition d'huile isolante se situe entre 5 et 15%.

9. Composition selon la revendication 1, dans laquelle les points d'ébullition de ladite fraction se situent dans une gamme de températures de 260° à 400°C.

10. Composition selon la revendication 1, dans laquelle les points d'ébullition de ladite fraction se situent dans une gamme de températures de 267° à 400°C.

11. Composition selon la revendication 1, dans laquelle les points d'ébullition de ladite fraction se situent dans une gamme de températures de 275° à 420°C.

12. Composition selon la revendication 1, dans laquelle les points d'ébullition de ladite fraction se situent dans une gamme de températures de 280°C à 400°C.
